

## UNITED STATES PATENT OFFICE

2,401,217

WAX COMPOSITION AND METHOD OF  
PREPARING THE SAME

Michael Berliney, Jersey City, Garfield Arthur Bowden, East Orange, and Jack Taylor Hohnstine, Short Hills, N. J., assignors, by mesne assignments, to Boyle-Midway Inc., New York, N. Y., a corporation of Delaware

No Drawing. Application November 4, 1942,  
Serial No. 464,512

5 Claims. (Cl. 106—219)

The invention relates to waxes and wax blends and the methods of preparing the same and is designed primarily to produce waxes using the minimum of natural waxes and wax-like materials in their composition.

With this object in view the invention consists in waxy compositions wherein paraffin wax may, by a special process, be intimately blended with rosins of the ester gum or polymerized types, stearic acid, stearates and certain animal, vegetable or mineral oils to form finished products suitable for coating compositions for waterproofing purposes.

For the purpose of waterproofing paper board containers designed for ammunition, food or the like, and for coating paper, we have developed a waxy composition which utilizes paraffins, a natural polymerized wood rosin, or a rosin of the ester gum type, stearic acid, a mineral oil, a vegetable oil and a stearate. The following formulas have been found suitable and are presented as exemplary:

(1)

|                                      | Lbs. |
|--------------------------------------|------|
| Paraffin—123 to 125° F.              | 57   |
| Paraffin—160 to 165° F.              | 25   |
| Rosin                                | 18   |
| Stearic acid single pressed          | 8    |
| Mineral oil 85° viscosity at 100° F. | 2    |
| Castor oil CP                        | 4    |
| Calcium stearate                     | 5    |

(2)

|                                      | Lbs. |
|--------------------------------------|------|
| Paraffin—123 to 125° F.              | 57   |
| Paraffin—160 to 165° F.              | 25   |
| Rosin                                | 18   |
| Stearic acid single pressed          | 8    |
| Mineral oil 85° viscosity at 100° F. | 2    |
| Soya bean oil blown                  | 4    |
| Calcium stearate                     | 5    |

(3)

|                                      | Lbs. |
|--------------------------------------|------|
| Paraffin—123 to 125° F.              | 57   |
| Paraffin—160 to 165° F.              | 25   |
| Rosin                                | 18   |
| Stearic acid single pressed          | 8    |
| Mineral oil 85° viscosity at 100° F. | 6    |
| Calcium stearate                     | 5    |

|                             | Lbs. |
|-----------------------------|------|
| Paraffin—123 to 125° F.     | 57   |
| Paraffin—160 to 165° F.     | 25   |
| Rosin                       | 18   |
| Stearic acid single pressed | 8    |
| Peanut oil                  | 6    |
| Calcium stearate            | 5    |

|                         | Lbs. |
|-------------------------|------|
| Paraffin—123 to 125° F. | 57   |
| Paraffin—160 to 165° F. | 25   |
| Rosin                   | 18   |
| Soya bean oil, raw      | 6    |
| Calcium stearate        | 5    |

|                             | Lbs. |
|-----------------------------|------|
| Paraffin—123 to 125° F.     | 57   |
| Paraffin—160 to 165° F.     | 25   |
| Rosin                       | 18   |
| Stearic acid single pressed | 8    |
| Fish oil                    | 6    |
| Calcium stearate            | 5    |

The process of preparing the finished wax from the above formulas is, for example, as follows:

In a gas fired iron kettle the full amount of rosin is placed and approximately one third to two thirds, depending upon the nature of the material to be treated with the composition, of the castor oil (Table 1) is added thereto, together with about one half of the stearic acid and the ingredients heated until thoroughly melted. A wooden paddle is used to stir the mixture until completely mixed. The temperature used for mixing and melting is within the range of from approximately 290 to 300° F.

When the formula shown in Table 2 is used in the above example the soya bean oil blown is substituted for the castor oil and it should be noted that Tables 1 and 2 call for a mineral oil as well as the vegetable oils.

In a separate steam jacketed mixing kettle the remaining stearic acid is placed and the entire amount of both paraffins added thereto whereafter the temperature is raised to within the range of approximately from 200 to 220° F. The remainder of the castor oil (Table 1) is then added together with the mineral oil. This mix-

ture is then agitated with a power agitator for about five minutes. At this point the molten rosin, stearic acid and castor oil mixture previously prepared is added slowly and with constant agitation. When all of the rosin mixture has been added agitation is continued for from five to ten minutes and the temperature adjusted to approximately 250° F. The five lbs. of calcium stearate is then added slowly and with constant agitation and maintenance of the temperature 10 at approximately 250° F.

For the formula shown in Table 2 in the above step soya bean oil blown is substituted for the castor oil.

Using the formulas in Tables 3, 4, 5 and 6 wherein only one oil, either animal, vegetable or mineral is used the following process applies.

The full amount of rosin is placed in a gas fired iron kettle and approximately one half of the oil is added thereto, together with about one half of the stearic acid and the mixture heated with stirring until thoroughly melted. The temperature used is within the range of from approximately 290 to 300° F.

In a separate steam jacketed mixing kettle the remainder of the stearic acid is placed and the entire amount of both paraffins added thereto whereafter the temperature is raised to within the range of from 200 to 220° F. The remainder of the oil is then added and the mixture then agitated with a power agitator for about five minutes. Following this the molten rosin, stearic acid and oil mixture previously prepared is added slowly with constant agitation, such agitation being continued for from five to ten minutes after all of the rosin mixture has been added. The temperature is adjusted to 250° F. and the calcium stearate added with constant agitation and maintenance of the 250° F. temperature.

The complete mixture is drawn off into molds and is a clear brown amber colored liquid which upon cooling becomes light straw color without surface or inner crystallization of the finished cake.

The finished product has the following characteristics:

|                       |                           |
|-----------------------|---------------------------|
| Softening point       | 142-150° F.               |
| Flash point           | 400°±5° F.                |
| Fire point            | 440°±5° F.                |
| Acid value            | 15-18                     |
| Saponification number | 25-47                     |
| Viscosity             | 91.4±5 seconds at 210° F. |
| Water absorption      | 3%±1%                     |
| Penetration           | 60-90%                    |

and shows no separation on reheating for seven days at 100° F.

We have found that the combination of stearic acid, rosin and paraffin produces a waxy product of the proper structure and that the permeability of the product is determined by use of the mineral, an animal or a vegetable oil, as is also the flexibility of the product, such oil, or oils, providing the proper gel formation. Waterproofing

properties naturally inherent in the ingredients are aided by the use of a stearate.

The resulting product is exceedingly adaptable for the protection of paper board containers by waterproofing and is also suitable for the similar treatment of wood and cloth and other porous or semiporous materials.

What we claim is:

1. A process for producing a wax coating composition comprising melting together an ester type of rosin, stearic acid, and vegetable oil, separately melting together stearic acid, paraffin, vegetable oil and mineral oil, mixing together the two molten mixtures with constant agitation, adding to the composite mixture calcium stearate and cooling the resultant mix, said final mix containing paraffin as the major ingredient in amount, said rosin comprising about one fourth the amount of said paraffin, said stearic acid comprising about one half the amount of said rosin and said stearate and oils each being less in amount than said stearic acid.

2. A wax coating composition, comprising a mixture of an ester type rosin, stearic acid and paraffin wax, said wax constituting the major ingredient in amount, said rosin comprising about one fourth the amount of said wax and the stearic acid comprising about one half the amount of said rosin.

3. A wax coating composition, comprising a mixture of an ester type rosin, stearic acid, calcium stearate, a vegetable oil, a mineral oil and paraffin wax, said wax constituting the major ingredient in amount, said rosin comprising about one fourth the amount of said wax, the stearic acid comprising about one half the amount of said rosin and said stearate and oils each being less in amount than said stearic acid.

4. A wax coating composition, comprising a mixture of an ester type rosin, stearic acid, calcium stearate, paraffin wax and an oil for imparting both permeability and flexibility to the product, selected from the group consisting of mineral, vegetable and fish oils, said wax constituting the major ingredient in amount, said rosin comprising about one fourth the amount of said wax, the stearic acid comprising about one half the amount of said rosin and said stearate and oil each being less in amount than said stearic acid.

5. A wax coating composition, comprising a mixture of an ester type rosin, stearic acid, paraffin wax, calcium stearate and a vegetable oil for imparting both permeability and flexibility to the product, said wax constituting the major ingredient in amount, said rosin comprising about one fourth the amount of said wax, said stearic acid comprising about one half the amount of said rosin and said stearate and oil each being less in amount than said stearic acid.

MICHAEL BERLINEY,  
GARFIELD ARTHUR BOWDEN,  
JACK TAYLOR HOHNSTINE.